



US010711351B1

(12) **United States Patent**  
Martin et al.

(10) **Patent No.:** US 10,711,351 B1  
(45) **Date of Patent:** Jul. 14, 2020

(54) **ELECTROLESS PLATING COMPOSITION FOR ELECTROLESS DEPOSITION OF ALUMINUM OR ALUMINUM ALLOY AND ARTICLE INCLUDING ELECTROLESS DEPOSITED ALUMINUM LAYER**

(71) Applicant: **HRL LABORATORIES, LLC**, Malibu, CA (US)

(72) Inventors: **John H. Martin**, Los Angeles, CA (US); **Joanna A. Kolodziejska**, Arcadia, CA (US); **John J. Vajo**, West Hills, CA (US); **Jason A. Graetz**, Calabasas, CA (US); **Christopher S. Roper**, Santa Monica, CA (US)

(73) Assignee: **HRL Laboratories, LLC**, Malibu, CA (US)

(\*) Notice: Subject to any disclaimer, the term of this patent is extended or adjusted under 35 U.S.C. 154(b) by 309 days.

(21) Appl. No.: **15/665,011**

(22) Filed: **Jul. 31, 2017**

**Related U.S. Application Data**

(62) Division of application No. 14/167,733, filed on Jan. 29, 2014, now Pat. No. 9,803,283.

(60) Provisional application No. 61/893,064, filed on Oct. 18, 2013.

(51) **Int. Cl.**

**C23C 18/16** (2006.01)  
**C23C 18/31** (2006.01)  
**C23C 18/48** (2006.01)  
**C23C 18/52** (2006.01)

(52) **U.S. Cl.**

CPC ..... **C23C 18/1687** (2013.01); **C23C 18/31** (2013.01)

(58) **Field of Classification Search**

None  
See application file for complete search history.

(56) **References Cited**

**U.S. PATENT DOCUMENTS**

|               |         |                |            |
|---------------|---------|----------------|------------|
| 2,446,331 A   | 8/1948  | Hurley         | C23C 16/06 |
| 3,462,288 A * | 8/1969  | Hellmann       | 427/595    |
| 3,635,761 A * | 1/1972  | Haag           | C23C 18/44 |
|               |         |                | 427/99.5   |
| 3,653,953 A * | 4/1972  | Grant, Jr.     | C23C 18/31 |
|               |         |                | 427/437    |
| 3,705,051 A * | 12/1972 | Kobetz et al.  | C03C 17/10 |
|               |         |                | 427/229    |
| 3,787,225 A   | 1/1974  | Roberts et al. |            |

(Continued)

**FOREIGN PATENT DOCUMENTS**

WO WO 2012/144518 A1 10/2012

**OTHER PUBLICATIONS**

Koura et al., "Electroless Plating of Aluminum from a Room-Temperature Ionic Liquid Electrolyte", Journal of the Electrochemical Society, 155(2):D155-D157, 2008.

(Continued)

*Primary Examiner* — Helene Klemanski

(74) *Attorney, Agent, or Firm* — Lewis Roca Rothgerber Christie, LLP

(57) **ABSTRACT**

An article includes an electroless deposited aluminum layer. The aluminum layer is deposited in an electroless plating composition. The composition includes an aluminum ionic liquid, a reducing agent, and an additive selected from the group consisting of a catalyst, an alloying element, and a combination thereof.

**6 Claims, 4 Drawing Sheets**



(56)

**References Cited**

## U.S. PATENT DOCUMENTS

- 5,160,422 A \* 11/1992 Nishimura ..... C23C 18/48  
106/1.22  
9,803,283 B1 \* 10/2017 Martin ..... C23C 18/1687  
10,190,227 B2 \* 1/2019 Ruan ..... C23C 30/00  
2005/0048210 A1 \* 3/2005 Siau ..... C23C 18/31  
427/372.2  
2006/0062902 A1 \* 3/2006 Sager ..... B22F 1/0018  
427/74  
2006/0251800 A1 \* 11/2006 Weidman ..... B82Y 30/00  
427/99.5  
2008/0187675 A1 8/2008 Scarpa et al.  
2009/0301894 A1 \* 12/2009 Ehlers ..... C23C 18/165  
205/170  
2011/0311822 A1 12/2011 Hao et al.

- 2014/0030635 A1 1/2014 Nakada et al.  
2015/0101935 A1 \* 4/2015 Chen ..... C25D 17/002  
205/208  
2016/0054487 A1 \* 2/2016 Cojocaru ..... C23C 18/31  
359/845  
2019/0186033 A1 \* 6/2019 Ruan ..... C23C 30/00

## OTHER PUBLICATIONS

- Shitanda et al., "Electroless plating of aluminum using diisobutyl aluminum hydride as liquid reducing agent in room-temperature ionic liquid", *Electrochima Acta* 54, 5889-5893, 2009.  
Tsuda et al., "Electrodeposition of Al-Zr Alloys from Lewis Acidic Aluminum Chloride-1-Ethyl-3-methylimidazolium Chloride Melt", *Journal of the Electrochemical Society*, 151(7):C447-C454, 2004.

\* cited by examiner

Fig. 1



Fig. 2



**Fig. 3**



Fig. 4



## 1

**ELECTROLESS PLATING COMPOSITION  
FOR ELECTROLESS DEPOSITION OF  
ALUMINUM OR ALUMINUM ALLOY AND  
ARTICLE INCLUDING ELECTROLESS  
DEPOSITED ALUMINUM LAYER**

**CROSS-REFERENCE TO RELATED  
APPLICATIONS**

This application is a divisional of U.S. application Ser. No. 14/167,733, filed on Jan. 29, 2014, now U.S. Pat. No. 9,803,283, which claims priority to and the benefit of U.S. Provisional Application No. 61/893,064, filed Oct. 18, 2013, the entire contents of both of which are incorporated herein by reference.

**STATEMENT REGARDING FEDERALLY  
SPONSORED RESEARCH OR DEVELOPMENT**

This invention was made with Government support under Contract No. W91CRB-10-C-0305 awarded by the US ARMY. The Government has certain rights in the invention.

**FIELD OF THE INVENTION**

The present disclosure relates to a method of electroless deposition of aluminum or aluminum alloy, an electroless plating composition, and an article including the same.

**INTRODUCTION**

Aluminum, due to its abundance and superior properties such as corrosion resistance, thermal and electric conductivity, or low density, has been used widely in applications such as electronics, packaging, construction, household items, toys, or transportation vehicles. In those applications, aluminum is used either as a sheet or foil that is relatively thick (e.g., about 1 cm or more), or a coating or film that is relatively thin (e.g., about 1 cm or less).

Aluminum is currently applied as a coating or thin film using methods such as aluminum cladding (a process where aluminum and another metal are bonded together by being rolled together at a suitable pressure and temperature), thermal or slurry spraying (where molten or semi-molten aluminum, or an aluminum containing slurry is sprayed onto a substrate), physical or chemical vapor deposition (where thin aluminum film is produced through condensation of a vaporized form of aluminum under high vacuum), or electrolytic deposition (also referred to as electrolytic plating, where electrical current is used to reduce dissolved aluminum cations to form an aluminum film on an electrode). However, each of the methods has some drawbacks and they are all limited to a substrate of simple geometry. For example, aluminum cladding is generally limited to flat sheets and difficult to apply to complex geometries. Thermal or slurry spraying also has limitation to the geometry of the substrate and requires line of sight for the coating to be deposited. In addition, the spraying methods tend to have non-uniformity issue and the product may contain contaminants from the process and therefore limiting the application of this method. Physical or chemical vapor deposition, on the other hand, requires expensive and specialized equipment, is conducted at a high temperature, and is only applicable to selected substrates with simple geometries. Electrolytic deposition of aluminum, when conducted in a solvent system, in addition to the drawback of using highly flammable solvents, can only be used to deposit pure alu-

## 2

minum. When using ionic liquid based aluminum alloy deposition, due to the low solution conductivity of aluminum or aluminum alloys, it is often difficult to plate alloy onto complex geometries, and also difficult to produce a coating of uniform thickness. In addition, this process requires very high power and unattainable for large parts. Besides, this process is only applicable to conductive substrates, and therefore, a non-conductive substrate has to be modified with a conductive layer prior to the electrolytic deposition.

Electroless deposition of aluminum has been explored in recent years. However, it is only limited to the deposition of pure aluminum coating on a glass plate or a copper sheet, and the rate of deposition is relatively slow (around 0.01 mg/cm<sup>2</sup>-minute).

**SUMMARY OF THE INVENTION**

An aspect of an embodiment of the present invention is directed toward a method for electroless deposition of aluminum on a substrate. Another aspect of an embodiment of the present invention is directed toward an electroless plating composition and an article including electroless deposited aluminum layer.

Additional aspects will be set forth in part in the description which follows and, in part, will be apparent from the description, or may be learned by practice of the presented embodiments.

30 A method for electroless deposition of aluminum on a substrate may include: activating the substrate; providing an aluminum ionic liquid; adding a reducing agent and an additive to the aluminum ionic liquid to form an electroless plating composition, wherein the additive may be one selected from the group consisting of a catalyst, an alloying element, and a combination thereof; and immersing the substrate in the electroless plating composition.

35 The reducing agent may be selected from alkali metal hydrides, alkaline earth metal hydrides, alenate salts of alkali metal, alenate salts of alkaline earth metal, borohydride salts, hydrided alkyl-metal compounds, or a combination thereof.

The reducing agent may be lithium hydride, di-isobutyl aluminum hydride, NaAlH<sub>4</sub>, LiBH<sub>4</sub> or NaBH<sub>4</sub>.

40 The aluminum ionic liquid may include 1-ethyl-3-methylimidazolium chloride, N-alkylpyridinium halides, N-alkylimidazolium halides, N,N'-alkylimidazolium halides, N-alkylpyrazolium halides, N, N'-alkylpyrazolium halides, bis(trifluoromethylsulfonyl) amide, tris(pentafluoroethyl) trifluorophosphate, trifluoroacetate, trifluoromethylsulfonate, dicyanoamide, tricyanomethide, tetracyanoborate, tetraphenylborate, tris(trifluoromethylsulfonyl) methide, thiocyanate, or a combination thereof.

45 The additive may include the catalyst, and the catalyst may be selected from the group consisting of TiCl<sub>2</sub>, TiCl<sub>3</sub>, TiCl<sub>4</sub>, ZrCl<sub>4</sub>, VCl<sub>3</sub>, NbCl<sub>5</sub>, CeCl<sub>3</sub> and combinations thereof.

The catalyst may be included from about 2 ppm to about 1 weight percent based on a total weight of the electroless plating composition.

50 The activating of the substrate may include: degreasing the substrate; etching the substrate utilizing a weak acid, strong acid, weak base, or strong base; and creating catalytic metal sites on the substrate for deposition.

55 The creating catalytic metal sites on the substrate for deposition may include depositing iron, palladium, silver, gold, ruthenium, rhodium, osmium, iridium, platinum, or combinations thereof on the substrate.

The creating catalytic metal sites on the substrate for deposition may include depositing palladium on the substrate utilizing physical vapor deposition, chemical vapor deposition, or a solution/suspension of palladium.

The substrate may include glass, metal, metal oxide, ceramic, organic material, or polymer.

The substrate may have a complex geometry, and the aluminum layer may be uniformly deposited on the substrate.

The method may further include adding particulates in the electroless plating composition prior to the immersing the substrate in the electroless plating composition, and the aluminum layer is deposited on the substrate with the particulates.

The particulates may include MgSi, SiC, CrC, TiC, BN, BC, diamond, metal, metal alloy, or a combination thereof.

The particulates may be about 10 nm to about 100 microns in diameter.

The method may further include removing the substrate to have a free standing aluminum layer.

The removing of the substrate may be conducted utilizing solvent dissolving, chemical etching, mechanical erasing, plasma discharging, electrical discharging, or thermal decomposing.

The additive may include the alloying element.

The alloying element may be selected from B, Mg, Sc, Ti, V, Cr, Mn, Fe, Co, Ni, Cu, Zn, Si, Ga, Ge, Y, Zr, Nb, Mo, Tc, Ru, Rh, Pd, Ag, Cd, In, Sn, Sb, Hf, Ta, W, Re, Os, Jr, Pt, Au, Tl, Pb, La, Ce, Nd, Sm, Ac, Th, U, Pu, or combinations thereof.

The alloying element may be included from about 0.01 atomic percent to about 95 atomic percent of the aluminum layer.

The additive may include the catalyst and the alloying element.

An article may include an electroless deposited aluminum layer, wherein the aluminum layer may include aluminum and less than about 1 weight percent of a metal element of a catalyst based on a total weight of the aluminum layer, the catalyst being selected from the group consisting of TiCl<sub>2</sub>, TiCl<sub>3</sub>, TiCl<sub>4</sub>, ZrCl<sub>4</sub>, VCl<sub>3</sub>, NbCl<sub>5</sub>, CeCl<sub>3</sub> and combinations thereof.

The aluminum layer may further include particulates.

The particulates may be selected from Mg<sub>2</sub>Si, SiC, CrC, TiC, BN, BC, diamond, metal, metal alloy, or a combination thereof.

The particulates may be about 10 nm to about 100 microns in diameter.

The aluminum layer may further include about 0.01 atomic percent to about 95 atomic percent of one or more alloying elements, the one or more alloying elements being selected from B, Mg, Sc, Ti, V, Cr, Mn, Fe, Co, Ni, Cu, Zn, Si, Ga, Ge, Y, Zr, Nb, Mo, Tc, Ru, Rh, Pd, Ag, Cd, In, Sn, Sb, Hf, Ta, W, Re, Os, Jr, Pt, Au, Tl, Pb, La, Ce, Nd, Sm, Ac, Th, U, Pu, or combinations thereof.

The aluminum layer may include amorphous, nanocrystalline, microcrystalline, multiphase, or mixed crystal size structure.

The aluminum layer may include a first layer of a first composition, and a second layer of a second composition different from the first composition.

The article may further include a substrate selected from glass, metal, metal oxide, ceramic, organic material, or polymer; and the aluminum layer may be uniformly deposited on the substrate.

The substrate may have a microtruss structure, or a complex shape.

A grain size of the aluminum may be less than 100 microns.

A grain size of the aluminum may be less than 10 microns.

A grain size of the aluminum may be less than 1 microns.

The aluminum layer may be less than 1 cm in thickness.

The aluminum layer may be less than 1 mm in thickness.

The aluminum layer may be less than 100 microns in thickness.

The aluminum layer may be less than 1 micron in thickness.

The article may consist essentially of the electroless deposited aluminum layer, the aluminum layer may further include about 0.01 atomic percent to about 95 atomic percent of one or more alloying elements, and the metal element of the catalyst may be included in about 2 ppm to about 1 wt % based on the total weight of the aluminum layer.

The one or more alloying elements may be selected from B, Mg, Sc, Ti, V, Cr, Mn, Fe, Co, Ni, Cu, Zn, Si, Ga, Ge, Y, Zr, Nb, Mo, Tc, Ru, Rh, Pd, Ag, Cd, In, Sn, Sb, Hf, Ta, W, Re, Os, Jr, Pt, Au, Tl, Pb, La, Ce, Nd, Sm, Ac, Th, U, Pu, or combinations thereof.

A grain size of the aluminum and/or the alloying element may be about 1 nm to about 100 nm.

The aluminum layer may further include particulates.

An electroless plating composition may include an aluminum ionic liquid; a reducing agent; and an additive selected from the group consisting of a catalyst, an alloying element, and a combination thereof.

#### BRIEF DESCRIPTION OF THE DRAWINGS

These and other features and advantages of the present invention will be better understood by reference to the following detailed description when considered in conjunction with the following drawings, in which:

FIG. 1 is a flow chart illustrating a method of electroless deposition of aluminum accordingly to one embodiment of the present invention;

FIG. 2 is a photograph image of an electroless plated microtruss manufactured according to the process of the Example;

FIG. 3 is an SEM image of the aluminum layer deposited on the microtruss of FIG. 2; and

FIG. 4 is an EDS spectrum of the aluminum layer deposited on the microtruss of FIG. 2.

#### DETAILED DESCRIPTION

Herein after, an “aluminum layer” may refer to a pure aluminum layer with less than 1 wt % of another element (such as an element of the catalyst), a layer of an aluminum-alloy, or a particulate containing aluminum or aluminum alloy layer. The term “electroless deposition” and “electroless plating” are used interchangeably. Expressions such as “at least one of,” when preceding a list of elements, modify the entire list of elements and do not modify the individual elements of the list. Further, the use of “may” when describing embodiments of the present invention refers to “one or more embodiments of the present invention.”

Referring to FIG. 1, a method for electroless deposition of aluminum layer on a substrate includes activating the substrate in act 101; providing an aluminum ionic liquid in act 103; adding a reducing agent and an additive to the aluminum ionic liquid to form an electroless plating composition in act 105; and immersing the substrate in the electroless plating composition to have an aluminum layer deposited on

the substrate in act 107. The additive may be a catalyst, one or more alloying elements, or particulates.

The substrate to be deposited with the aluminum layer may be made of any suitable material that can withstand submersion in the ionic liquid. Examples of such suitable materials include, but not limited to, glass, metal, metal oxide, ceramic, organic material, or polymer. The substrate may have any desired geometry, including a simple geometry such as a flat sheet, or a more complex geometry, such as a cube, a sphere, a pipe, or a microtruss structure. A microtruss structure is an ordered three-dimensional structure at the micrometer scale. A microtruss structure includes a plurality of first truss elements extending along a first direction; a plurality of second truss elements extending along a second direction; and a plurality of third truss elements extending along a third direction. The first, second, and third truss elements interpenetrate each other at a plurality of nodes to form a continuous material (see FIG. 2). U.S. Pat. No. 7,382,959 B1 (Optically Oriented Three-Dimensional Polymer) discloses such microtruss structures and methods of making the same, the entire content of which is incorporated herein by reference.

The activating of the substrate may include degreasing the substrate; etching the substrate utilizing a weak acid, strong acid, weak base, or strong base; and creating catalytic metal sites on the substrate for deposition, but the present invention is not limited thereto. For example, one or more of the acts may not be included in the activating of the substrate. For example, the degreasing of the substrate may not be included in the activating of the substrate.

The degreasing of the substrate may be conducted by washing the substrate in a solution of a soap, a surfactant, or a weak or a strong base solution. In one embodiment, a substrate is degreased using NaOH. By using a weak acid, a strong acid, a weak base, or a strong base, the etching of the substrate further removes any surface contaminants off the substrate, and creates desired surface morphology of the substrate. In one embodiment, a substrate is etched using 10% HCl. The creating of catalytic metal sites on the substrate for deposition may be conducted using physical vapor deposition, chemical vapor deposition, or a solution/suspension deposition of the catalytic metal. Suitable catalytic metals may be any metal that can promote metal hydride decomposition on the substrate. Examples of suitable catalytic metals include iron, or noble metals such as palladium, silver, gold, ruthenium, rhodium, osmium, iridium or platinum. In one embodiment, a polymer substrate is first etched using a base to create small holes on the polymer substrate; a colloidal suspension of palladium particles is then utilized to deposit palladium particles on the substrate, especially in the etched holes on the substrate, to create the catalytic metal sites. However, the present invention is not limited thereto. For example, the creating of catalytic metal sites on the substrate may not be included in the activating of the substrate.

The aluminum ionic liquid may include aluminum halide (such as aluminum chloride) and an ionic liquid of another salt, mixed at a suitable ratio. Suitable ionic liquids of another salt may include, but not limited to, 1-ethyl-3-methylimidazolium chloride, N-alkylpyridinium halides, N-alkylimidazolium halides, N,N'-alkylimidazolium halides, N-alkylpyrazolium halides, N,N'-alkylpyrazolium halides, bis(trifluoromethylsulfonyl) amide, tris(trifluoromethylsulfonyl-trifluorophosphate, trifluoroacetate, trifluoromethylsulfonate, dicyanoamide, tricyanomethide, tetracyanoborate, tetraphenylborate, tris(trifluoromethylsulfonyl)methide, thiocyanate, or a combination thereof. In one

embodiment, aluminum chloride and 1-ethyl-3-methylimidazolium chloride are mixed at 2:1 molar ratio to make the aluminum ionic liquid.

The reducing agent may be any suitable compound that can give electrons to metal ions to deposit the reduced metal on the substrate. Examples of suitable reducing agent include alkali metal hydrides, alkaline earth metal hydrides, alanate salts of alkali metal, alanate salts of alkaline earth metal, borohydride salts, hydrided alkyl-metal compounds, and a combination thereof. In one embodiment, lithium hydride (LiH), LiAlH<sub>4</sub>, di-isobutyl aluminum hydride (DIBAH), NaAlH<sub>4</sub>, LiBH<sub>4</sub> or NaBH<sub>4</sub> is used as the reducing agent. The reducing agent may be added at a suitable amount. The amount of the reducing agent controls the electroless plating rate and the thickness of the deposit. That is, the more the reducing agent, the faster the electroless deposition, and the thicker the deposit. For example, the reducing agent may be added at a concentration of about 0.1 to about 5 M in the aluminum ionic liquid. In one embodiment, the reducing agent is added at a concentration of 0.5, 1.0, or 2.0 M in the aluminum ionic liquid.

The additive may be a catalyst, an alloying element, or a combination thereof. The additive may further include particulates. In the context according to embodiments of the present invention, a catalyst is a compound that can promote the reduction of aluminum ions and other metal elements to form a metallic deposit on the substrate when added at a small amount to the electroless plating composition. Suitable catalysts include, but not limited to, metals, metal powders, or metal salts such as TiCl<sub>2</sub>, TiCl<sub>3</sub>, TiCl<sub>4</sub>, ZrCl<sub>4</sub>, VCl<sub>3</sub>, NbCl<sub>5</sub>, or CeCl<sub>3</sub>. The catalyst may be added at a suitable amount. In one embodiment, the catalyst is added at about 2 ppm to about 1 wt % based on the total weight of the electroless plating composition. The deposition rate and the quality of the deposited layer may be improved with the addition of the catalyst. In one embodiment, when using di-isobutyl aluminum hydride as a reducing agent without a catalytic additive, no deposition occurred on a micro-truss substrate, while the deposition proceeded quickly for the same solution when a catalytic additive was added. In another embodiment, when using LiH as a reducing agent without a catalyst, aluminum was deposited on a microtruss substrate, but did not have acceptable cohesion and the aluminum layer flaked off easily. However, when a new solution of the same composition with the addition of an catalytic additive was used for the deposition, a coherent white deposit was deposited on the microtruss.

The additive may be one or more alloying elements. An alloying element may enhance the thermal or mechanical properties of the electroless deposited aluminum-alloy (such as strength or ductility), the microstructure of electroless deposited aluminum-alloy, and the process, particularly, the rate of the electroless deposition. For example, the alloying element may lead to an autocatalytic deposition process or enhance such a process. The alloying element may lead to the formation of nanocrystalline structure rather than micro-crystalline structure of the deposited layer.

The alloying elements may be any suitable metal elements that can form a corresponding metal hydride in the ionic liquid (through reaction with the reducing agent), and the corresponding metal hydride can also be decomposed to be co-deposited with aluminum on the substrate through the electroless deposition process. For example, MgCl<sub>2</sub> may be reduced by LiH through the favorable metathesis reaction 2LiH+MgCl<sub>2</sub>=2LiCl+MgH<sub>2</sub>. MgH<sub>2</sub> may then be decomposed and Mg is deposited on the substrate. However, due to the higher stability of LiCl, it may not be possible to use

$\text{MgH}_2$  to reduce  $\text{LiCl}$  to  $\text{LiH}$  for electroless deposition of  $\text{Li}$ . When a suitable catalyst is utilized, even a metal whose hydride that is relatively hard to be reduced may also be utilized as an alloying element to aluminum, due to the catalytic effect. For example,  $\text{TiH}_4$  is highly unstable and likely to be reduced and deposited on a substrate while  $\text{TiH}_2$  is generally more stable under normal conditions and may not be electrolessly deposited on the substrate. However, when a suitable catalyst, such as  $\text{TiCl}_3$ , is added to the ionic liquid, it is even possible to electrolessly deposit  $\text{Ti}$  from  $\text{TiH}_2$ .

Suitable alloying elements include, but not limited to,  $\text{B}$ ,  $\text{Mg}$ ,  $\text{Sc}$ ,  $\text{Ti}$ ,  $\text{V}$ ,  $\text{Cr}$ ,  $\text{Mn}$ ,  $\text{Fe}$ ,  $\text{Co}$ ,  $\text{Ni}$ ,  $\text{Cu}$ ,  $\text{Zn}$ ,  $\text{Si}$ ,  $\text{Ga}$ ,  $\text{Ge}$ ,  $\text{Y}$ ,  $\text{Zr}$ ,  $\text{Nb}$ ,  $\text{Mo}$ ,  $\text{Te}$ ,  $\text{Ru}$ ,  $\text{Rh}$ ,  $\text{Pd}$ ,  $\text{Ag}$ ,  $\text{Cd}$ ,  $\text{In}$ ,  $\text{Sn}$ ,  $\text{Sb}$ ,  $\text{Hf}$ ,  $\text{Ta}$ ,  $\text{W}$ ,  $\text{Re}$ ,  $\text{Os}$ ,  $\text{Jr}$ ,  $\text{Pt}$ ,  $\text{Au}$ ,  $\text{Tl}$ ,  $\text{Pb}$ ,  $\text{La}$ ,  $\text{Ce}$ ,  $\text{Nd}$ ,  $\text{Sm}$ ,  $\text{Ac}$ ,  $\text{Th}$ ,  $\text{U}$ ,  $\text{Pu}$ , or combinations thereof. In one embodiment, one or more alloying elements are utilized. In one embodiment, an  $\text{Al}-\text{B}$  alloy is electrolessly deposited on a substrate. In another embodiment, an  $\text{Al}-\text{Cu}-\text{Ti}-\text{Zr}$  alloy is electrolessly deposited on a substrate.

The alloying element may be added as an anhydrous metal halide salt of the alloying element or added by electrolytic dissolution of the selected metal anode into the aluminum ionic liquid. The alloying element may be included in a suitable amount according to the desired structure and property of the deposited aluminum layer. In one embodiment, one or more alloying elements are included from about 0.01 atomic fraction (at. %) to about 95 atomic percent of the deposited aluminum alloy layer, while the amount of all the elements of the deposited aluminum alloy layer adds up to 100 at. %. For example, one or more alloying elements are included from about 0.5 atomic percent to about 90 at. %, or from about 5 atomic percent to about 50 atomic percent of the deposited aluminum alloy layer.

The additive may further include particulates that are co-deposited with aluminum to form a particulate containing aluminum layer on the substrate. Suitable particulates may be about 10 nm to about 100 microns in diameter, and may enhance the mechanical property such as strength, surface roughness, surface energy, wearing, and aesthetics of the deposited particulate containing aluminum layer. Suitable particulates include, but not limited to,  $\text{Mg}_2\text{Si}$ ,  $\text{SiC}$ ,  $\text{CrC}$ ,  $\text{TiC}$ ,  $\text{BN}$ ,  $\text{BC}$ , diamond, metal, metal alloy, or a combination thereof. The particulates may be included in a suitable amount to provide the desired improvements or enhancements of the deposited particulate containing aluminum layer. In one embodiment, particulates are included in about 0.1 wt % to about 10 wt % based on the total weight of the deposited aluminum layer including the particulates.

In one embodiment, the additive is the catalyst. In another embodiment, the additive is the one or more alloying elements. In yet another embodiment, the additive is the catalyst, the one or more alloying elements, and the particulates, each included at a suitable amount.

After the electroless plating composition is prepared, the activated substrate is immersed in the electroless plating composition. The electroless deposition of aluminum is carried out in a moisture-free and oxygen-free environment.

During deposition, bubbles may be observed around the deposited substrate, indicating gas release being part of the deposition process. Without being bound by any particular theory, it is believed that the dissolved metal ions (e.g., from aluminum halide such as aluminum chloride) get hydrogenated through an exchange reaction with the reducing agent and form an unstable intermediate metal hydride (e.g., aluminum hydride, or aluminum-metal hydride). The intermediate metal hydride such as aluminum hydride, or alu-

minum-metal hydride is then deposited on the substrate through the catalyzed decomposition of the metal hydride at the activated substrate surface, resulting in the deposition of metal and release of hydrogen gas. For example, the catalytic metal on the catalytic metal sites of the activated substrate may initiate the deposition of aluminum or aluminum-metal alloy by promoting initial metal hydride decomposition. The reaction then proceeds auto-catalytically on the surface of the growing film (e.g., the deposited metal promotes additional deposition of aluminum or aluminum alloys). As the formed metal hydrides decompose at the surface of the substrate, the film growth may be an epitaxial type of growth, but is not limited thereto. The catalytic additives are believed to help destabilize the metal hydrides and encourage metal hydride decomposition which results in deposition of the metal on the substrate surface and the growth of the metal film. As a result, a layer of aluminum, aluminum-alloy, or particulate containing aluminum layer is deposited on the substrate. The electroless deposition may be conducted in room temperature or at a temperature lower than 200° C. To enhance the rate of deposition and the uniformity of the deposited layer on a complex shaped substrate, agitation may be provided during the electroless deposition process. Agitation may ensure replenishment of chemistry such as reducing agent at the surfaces of the substrate being deposited.

The rate of deposition and the thickness of the layer deposited on the substrate depend on the amount of the reducing agent. The more the reducing agent added, the faster the deposition. The process continues until the desired thickness is attained, or all the reducing agent is consumed.

The structure and properties of the deposit may be altered based on the surface condition of the substrate, speed of reaction, temperature, alloying elements and other reactants involved in the deposition. For example, increasing the temperature may increase the rate of metal hydride formation and decomposition and therefore increase the plating rate. A faster plating rate may decrease the grain size of the deposit. Certain alloying elements may also decrease the grain size when co-deposited.

In one embodiment of the present invention, a plurality of aluminum layers are sequentially electrolessly deposited on a substrate. A first layer is deposited by immersing the activated substrate in a first electroless plating composition. After the desired amount of aluminum layer is deposited on the substrate, the substrate is removed from the first electroless plating composition and immersed in a second electroless plating composition to have a second layer deposited thereon. The first and second electroless plating compositions may be different, but are not limited thereto. In one embodiment, a first layer of pure aluminum is first deposited on a substrate, and a second layer of an aluminum alloy is then deposited on the pure aluminum layer. Additional layers may be deposited in this fashion.

Once deposition is completed for a substrate and the substrate is removed from the electroless plating composition, depleted chemicals may be added and contaminants may be removed (such as through filtering), and the electroless plating composition may be reused for deposition to other substrates. Because substrates made of different materials may be deposited using similar procedures, an electroless deposition production line may be used to electrolessly deposit an aluminum layer on different substrates.

In one embodiment of the present invention, the substrate where the aluminum layer is deposited on may be further removed to have a free standing aluminum layer. The substrate may be removed utilizing any suitable method,

such as mechanical, chemical, or thermal methods. For example, the substrate may be removed through solvent dissolving, chemical etching, mechanical erasing, plasma discharging, electrical discharging, or thermal decomposing. In one embodiment of the invention, the substrate is a microtruss made of a polymer material. After an aluminum layer, an aluminum-alloy layer or a particulate containing aluminum layer has been formed on the microtruss substrate using electroless deposition, the polymer may be removed through solvent etching, and leaving a stand-alone aluminum based hollow microtruss structure. In another embodiment of the invention, the substrate is a plastic mold. The mold may be dissolved, melted, or reused after the aluminum layer has been electrolessly deposited on the mold substrate. In one embodiment, an electroless deposited layer is slipped off the mold to have a stand-alone aluminum based structure.

In yet another embodiment, the substrate is a carrier web made of a suitable material as described previously. After electroless deposition, the deposited layer is separated from the carrier web to provide a foil of pure aluminum, a foil of aluminum alloy, or a particulate containing aluminum foil. The carrier web may be reused. In one embodiment, the electroless deposition is a continuous process, with the substrate passing through multiple stations. For example, the substrate passes through a first station with a set of chemical baths to activate the substrate. The activated substrate then passes through a second station with a bath containing the electroless plating composition. The concentration of each ingredient forming the electroless plating composition, the size of the bath, and the amount of time the substrate stays in this second station may be adjusted according to the desired thickness of the deposited aluminum layer. The substrate then may pass through a third station where the deposited aluminum layer is separated from the substrate, wound into a roll, and the substrate free of the deposited layer is sent back to the first station. Reel-to-reel thin film production for pure aluminum foil, aluminum alloy foil, or particulate containing aluminum foil may be manufactured this way.

An electroless plating composition may include an aluminum ionic liquid; a reducing agent; and an additive selected from the group consisting of a catalyst, an alloying element, and a combination thereof.

An article manufactured using the method of electroless deposition of aluminum as described above may include an aluminum layer, and the aluminum layer may include aluminum and less than about 1 wt % of a metal element of a catalyst based on a total weight of the aluminum layer. The catalyst may be  $TiCl_2$ ,  $TiCl_3$ ,  $TiCl_4$ ,  $ZrCl_4$ ,  $VCl_3$ ,  $NbCl_5$ , or  $CeCl_3$ . The aluminum layer may further include particulates, selected from  $MgSi$ ,  $SiC$ ,  $CrC$ ,  $TiC$ ,  $BN$ ,  $BC$ , diamond, metal, metal alloy, or a combination thereof. The particulates may be about 10 nm to about 100 microns in diameter.

The aluminum layer may further include one or more alloying elements. For example, the aluminum layer may include  $B$ ,  $Mg$ ,  $Sc$ ,  $Ti$ ,  $V$ ,  $Cr$ ,  $Mn$ ,  $Fe$ ,  $Co$ ,  $Ni$ ,  $Cu$ ,  $Zn$ ,  $Si$ ,  $Ga$ ,  $Ge$ ,  $Y$ ,  $Zr$ ,  $Nb$ ,  $Mo$ ,  $Tc$ ,  $Ru$ ,  $Rh$ ,  $Pd$ ,  $Ag$ ,  $Cd$ ,  $In$ ,  $Sn$ ,  $Sb$ ,  $Hf$ ,  $Ta$ ,  $W$ ,  $Re$ ,  $Os$ ,  $Ir$ ,  $Pt$ ,  $Au$ ,  $Tl$ ,  $Pb$ ,  $La$ ,  $Ce$ ,  $Nd$ ,  $Sm$ ,  $Ac$ ,  $Th$ ,  $U$ ,  $Pu$ , or combinations thereof. The one or more alloying elements may be included at about 0.01 atomic percent to about 95 atomic percent based on the total atoms of the aluminum layer. When one or more alloying elements are included, microstructure of the deposited aluminum layer may include amorphous, nanocrystalline, microcrystalline, multiphase, or mixed crystal size structure. A grain size of the deposited aluminum layer may be less than 100 microns,

less than 10 microns, less than 1 micron, or about 1 nm to about 100 nm. A thickness of the deposited aluminum layer may be about 1 cm or less, about 1 mm or less, about 100 microns or less, or about 1 micron or less.

5 The alloying elements may strengthen the mechanical properties of the deposited aluminum layer. Multiple layers of aluminum or aluminum alloys may be deposited on one substrate, each having different composition, or provide a different function. For example, a layer closer to the substrate may have higher mechanical strength, while a layer closer to the free surface may have better abrasion resistance.

10 The method of electroless deposition of aluminum according to embodiments of the present invention may be used to create an aluminum coating or an aluminum-alloy coating on a substrate, or a free standing aluminum or aluminum-alloy structure with the substrate removed. The electroless deposited aluminum layer may form a decoration layer, a reflective coating layer (particularly suitable for complex geometries), a mirror, a wire bonding site for electrical connectors, a sacrificial corrosion resistant coating, a corrosion/wear coating (particularly suitable for complex geometries such as pipelines), or a wear resistant coating (particularly for non-conductive plastic materials). 15 The electroless deposited aluminum layer may be further anodized or dyed. The electroless deposited aluminum layer may also be used to form electronic materials, reel-to-reel coating of materials, or a diffusion coating where a coating is first applied on the surface of a substrate, and the coating later on diffuses into the substrate, for high performance applications such as super alloys with non-line of site limitations.

20 The following Example is provided for illustrative purpose only, and does not limit the scope of the present invention.

#### Example

25 A  $1\text{ cm}^3$  polymer microtruss was used as a substrate for electroless plating. The polymer microtruss was activated using standard commercial solutions for the electroless deposition of metals onto plastics. This included etching followed by activation in a colloidal palladium solution. The sample was allowed to dry and then placed into an argon filled glove box with oxygen content of less than 20 ppm.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9

**11**

from the underlying microtruss). The EDS spectrum also shows a trace amount of Ti, which may come from the  $TiCl_3$  as the catalyst.

While certain embodiments of the present invention have been illustrated and described, it is understood by those of ordinary skill in the art that certain modifications and changes can be made to the described embodiments without departing from the spirit and scope of the present invention as defined by the following claims, and equivalents thereof.

What is claimed is:

1. An electroless plating composition, comprising:  
an aluminum ionic liquid;  
a reducing agent; and  
an additive selected from the group consisting of a catalyst, an alloying element, and a combination thereof,  
wherein the additive comprises the catalyst, and the catalyst is selected from the group consisting of  $TiCl_2$ ,  $TiCl_3$ ,  $TiCl_4$ ,  $ZrCl_4$ ,  $VCl_3$ ,  $NbCl_5$ ,  $CeCl_3$  and combinations thereof.
2. The electroless plating composition of claim 1, wherein the reducing agent is selected from the group consisting of alkali metal hydrides, alkaline earth metal hydrides, alanate

**12**

salts of alkali metal, alanate salts of alkaline earth metal, borohydride salts, hydrided alkyl-metal compounds, and combinations thereof.

3. The electroless plating composition of claim 1, wherein the reducing agent is lithium hydride, di-isobutyl aluminum hydride,  $NaAlH_4$ ,  $LiBH_4$  or  $NaBH_4$ .

4. The electroless plating composition of claim 1, wherein the aluminum ionic liquid comprises 1-ethyl-3-methylimidazolium chloride, N-alkylpyridinium halides, N-alkylimidazolium halides, N,N'-alkylimidazolium halides, N-alkylpyrazolium halides, N,N'-alkylpyrazolium halides, bis(trifluoromethylsulfonyl) amide, tris(pentafluoroethyl) trifluorophosphate, trifluoromethylsulfonate, dicyanoamide, tricyanomethide, tetracyanoborate, tetraphenylborate, tris(trifluoromethylsulfonyl) methide, thiocyanate, or a combination thereof.

5. The electroless plating composition of claim 1, further comprising particulates about 10 nm to about 100 microns in diameter and/or selected from  $MgSi$ ,  $SiC$ ,  $CrC$ ,  $TiC$ ,  $BN$ ,  $BC$ , diamond, metal, metal alloy, and combinations thereof.

6. The electroless plating composition of claim 1, wherein the additive further comprises the alloying element.

\* \* \* \* \*